

## UNITED STATES PATENT OFFICE.

HERMANN MÜLLER, OF HERISAU, SWITZERLAND, ASSIGNOR TO THE FIRM AKTIEN-  
GESELLSCHAFT CILANDER, OF HERISAU, SWITZERLAND.

## METHOD FOR PRODUCING PATTERN EFFECTS IN FABRICS.

No Drawing. Application filed February 25, 1926, Serial No. 90,706, and in Germany January 20, 1926.

Pattern effects in the texture of fabrics are as a rule produced by embroidering smooth fabrics or by weaving so-called effect-yarns into certain parts of the fabric 5 during the manufacture of the latter. It has also been proposed to obtain a pattern effect by carbonizing the cotton by means of an acid in certain parts of mixed fabrics.

It has now been found that pattern effects 10 in the texture of mixed fabrics composed of animal fibres (for instance silk) and of vegetable fibres (for instance cotton) may be produced if such fabrics are treated in certain places with such alkalis which only destroy the animal fibres of the mixed fabric but not the vegetable fibres. In this manner 15 the destruction of the animal fibres in certain places produces pattern effects in the texture of mixed fabrics, inasmuch as in 20 those parts in which the animal fibres have been destroyed and removed only the vegetable fibres remain, whilst in the other parts the vegetable as well as the animal fibres are still present.

25 The manner in which the two different fibres are arranged in the texture of the fabric is of no principal importance for producing pattern effects; the animal fibres may be contained in the warp threads and the 30 vegetable fibres in the weft threads or vice versa or both may be contained in the warp as well as in the weft threads.

The character of the produced effect, however, depends on the arrangement of the two 35 different fibres and on their binding in the fabric as well as on the pattern which has been printed on the fabric with an alkali.

By previous or subsequent dyeing of the 40 mixed fabrics or by a simple bleaching or by printing the fabric with colours or by mordanting or like measures the most varied colour combinations may be obtained. The invention is not restricted to the use of a fabric composed of one sort of vegetable 45 fibres and one kind of animal fibres, fabrics may be treated which are composed of mixtures of several vegetable and animal fibres.

*Example.*

50 A fabric is manufactured the warp of which consists, for instance, of cotton and the weft of floret silk and cotton. Thereupon the fabric is bleached and dried and an alkaline gum thickening is printed on certain parts of the fabric, the latter being

thereupon dried and steamed to cause the alkali to penetrate well into the silk. Then the alkaline solution of gum together with the silk threads destroyed by it are removed by washing, whereby parts in the fabric are 60 formed which do no longer contain silk and other parts in which silk is still present. The latter parts form the patterns in the texture of the fabric.

On the other hand, according to the character of the designs which are utilized when printing with alkali pattern effects in the texture of a fabric may also be obtained with which those parts of the fabric produce the pattern effect in which the silk has 65 been removed by mordanting whilst the other parts of the fabric in which silk as well as cotton are still present form the ground.

70 On such a fabric provided with patterns 75 the most varied colour combinations may be obtained by utilizing special dyes for vegetable and animal fibres whereby only one kind of fibres or both are dyed.

I claim:

1. A method for producing pattern effects 80 in the texture of fabrics, which consists in printing a pattern on a mixed fabric of warp and weft threads only composed of animal and vegetable fibres by means of an alkaline paste, steaming the printed fabric, and washing it thereafter thereby producing the same pattern on both sides of the fabric in the original weave.

2. A method of producing pattern effects 85 in woven fabrics of animal and vegetable threads composed of untreated warp and weft threads only, which comprises printing a pattern on such a smooth fabric irrespective of any thread arrangement of the fabric, with an agent destructive of one type of threads, and washing out the said agent and the portions of the threads destroyed thereby producing the same pattern on both sides of the fabric in the original weave.

3. A method of producing pattern effects 90 in woven fabrics composed of untreated warp and weft threads only, one set of threads being of animal origin and the other set of threads of vegetable origin, which 95 comprises printing a pattern on such fabric with a substance that destroys one type of threads and not the other type of threads, and washing out said substance and the destroyed portions of the threads there-

by producing the same pattern on both sides of the fabric in the original weave.

4. A method of producing pattern effects in woven fabrics having warp and weft threads only, said fabric having threads of animal origin and threads of vegetable origin, comprising printing on one face of said fabric a pattern with a substance for destroying one kind of threads while leaving

the other kind of threads, said substance and pattern being applied to the fabric irrespective of any particular grouping of the threads in the weave thereby producing the same pattern on both sides of the fabric in the original weave. 10

In testimony whereof, I have signed my name to this specification.

HERMANN MÜLLER. 15